

# UNITED STATES PATENT OFFICE.

KENICHI MIYAZAKI, OF TOKYO, JAPAN.

## PROCESS OF TREATING TIN-PLATE FOR CANNED PROVISIONS.

1,148,851.

Specification of Letters Patent.

Patented Aug. 3, 1915.

No Drawing.

Application filed July 28, 1913. Serial No. 781,643.

To all whom it may concern:

Be it known that I, KENICHI MIYAZAKI, a subject of the Emperor of Japan, residing at No. 3 Koyamacho, Mita, Shiba-Ku, city of Tokyo, Empire of Japan, professor, have invented new and useful Improvements in Processes of Treating Tin-Plate for Canned Provisions, of which the following is a specification.

10 This invention relates to an improved process for coating the surface of tin plate used in the manufacture of cans, etc., for canned provisions with a mixture of raw lacquer and shellac, so as to render it proof against acid liquids, alkali and tannin in order to prevent its corrosion or dissolution through physical changes. At the same time, the coating prevents discoloration of the contents such as foods, shell fish, lobster, 20 crab, etc., which possess more or less acidity or alkalinity and which act so deterioratingly upon the metal surface as to cause chemical changes if they are packed in an ordinary tin can.

25 In carrying out my invention, I employ as a base of coating, compounds of raw lacquer and shellac, the preparation of which consists in first refining a raw lacquer, as for instance won from the lacquer-tree, 30 botanically known as "*Rhus vernicifera*", stirring gently, removing the greater part of the moisture, and other impurities, until desired hardness is reached, then adding thereto a certain quantity of dissolved shellac, and after thorough mixture, passing the 35 mass through a suitable filter, preferably through cotton. The mixture thus prepared is now fit for use.

The surface of an ordinary tin plate upon 40 which my said mixture is to be applied should be perfectly cleaned. For this purpose, I prepare a piece of clean rag or cloth, preferably soaked with a diluted alkali liquid in order to wipe off all the greasy 45 matters adhering to the surface of the tin plate, whereafter I wipe the plates with a piece of clean cloth or rag soaked in an acid in order to remove or neutralize the alkali previously used, after which the plate is 50 wiped carefully with some alcohol-soaked cloth to remove the moisture. The plate which is now cleaned will be then heated to a temperature of preferably from 50 to 60 degrees C. At this temperature the plate 55 is now carefully painted with the aforescribed mixture of lacquer and shellac spread

evenly over the heated surface. The painted plate will then be brought into a metallic frame, which is adapted to carry or hold several sheets of such painted plates for 60 the purpose of conveying them all at the same time into a closed wet chamber containing preferably from 75 to 95% of moisture (temperature of this room must not be lower than 10 degrees C.), where they are 65 allowed to remain for about 24 hours. This will make the painted material gradually dry and adhere. The frame carrying several sheets of the painted plates is now taken out of the wet chamber and passed into the 70 closed dry chamber, where they are heated for about 1½ to 2 hours to a temperature of preferably from 120 to 180 degrees C. By this final treatment, all the volatile organic substances contained in the mixture will be 75 evaporated, leaving a very brilliant goldish layer of coating firmly adhering to the surface of the tin plate, but bearing no offensive smell characteristic of the lacquer.

The coating adhering to the surface of 80 the tin plate is lasting and can not be removed. Even the bending of the plate up and down repeatedly can not remove the coating, which is of great advantage in the operation of can-making, because the punching, shearing, or flanging action of the machinery would have no effect on the part of the coating.

I have found that my coating withstands 85 a temperature of 200 degrees C., and, therefore, the high grade sterilization of canned goods on 120 degrees, or up, can be effectively carried out without deteriorating the contents of the cans.

Lobster and crab for instance, if packed in 90 an ordinary can, turn black very frequently, which defect is entirely obviated by my present invention.

Having now particularly described and ascertained the nature of my said invention, 100 and in what manner the same is to be performed, I declare that what I claim is:—

1. Process for producing lacquered tin plate especially for canning purposes consisting in cleaning the tin plate, coating 105 the same with a lacquer readily solidifying under constant stirring and containing a small percentage of shellac or varnish, treating the coated plate within a humid chamber and finally heating and drying the same 110 at a temperature of 120-180° C.

2. Process for producing lacquered tin

- plate, especially for canning purposes consisting in cleaning the tin plates with diluted alkali, neutralizing the alkali, treating the plate with alcohol and coating the same with 5 lacquer readily solidifying under constant stirring and containing a small percentage of shellac or varnish treating the plate within a humid chamber and finally heating and

drying the same at a temperature of 120-180° C.

In testimony whereof I affix my signature in presence of two witnesses.

KENICHI MIYAZAKI.

Witnesses:

GENJI KURIBARA,  
HARNTADA YASUMURA.